

Jan. 24, 1939.

C. J. TOLL

2,144,904

ANNEALING

Filed Feb. 21, 1935

Fig. 2.



Fig. 1.



Inventor:  
CARL J. TOLL,  
by *Usina & Rauber*  
his Attorneys.

## UNITED STATES PATENT OFFICE

2,144,904

## ANNEALING

Carl J. Toll, Worcester, Mass., assignor to The American Steel and Wire Company of New Jersey, a corporation of New Jersey

Application February 21, 1935, Serial No. 7,618

1 Claim. (Cl. 148—16)

This invention relates in general to annealing, and is particularly concerned with box or pot annealing, one of the objects being to pot anneal high carbon steel, wire or strip. Other objects 5 may be inferred.

According to the invention, wire is loaded onto an annealing pot and supported in spaced relationship respecting the entire inside of the latter during the annealing operation. This is done to 10 permit the gases enclosed in the pot to circulate more freely. Granular or porous carbonaceous material, such as charcoal, is then arranged in the pot so that the gases may contact therewith during the annealing operation. All leaks between the inside and outside of the pot are then 15 sealed with carbonaceous material, and a cover is provided so as to protect it from the furnace atmosphere.

Annealing is conducted in the usual manner 20 after the above acts have been performed. No appreciable decarburization of the charge will occur during this operation.

In the accompanying drawing, Figure 1 is a cross-section and Figure 2 a vertical section of an 25 annealing pot that is expressly designed to accommodate the practice which has been described.

This drawing shows an annealing pot 1 that is distinguished by being of somewhat larger diameter than the usual pot and by having a top 30 providing at least two closure seats 2 and 3. Also, the pot has an apertured internal shell 4 spaced from its outside, this shell being adapted to position the required granular or porous material 35 between it and the inside of the walls of the pot. This shell is provided with outwardly extending flanges 5, which serve to maintain the shell and pot in concentric relation, and apertures 5a, so 40 that at least a portion of the gases enclosed by the pot can circulate through and mingle with the carbonaceous material contained therein. The diameter of this shell is such as to permit loading of coils of wire 6.

The coils of wire 6 are carried by a work support 7 of the character described and claimed by 45 my Patent No. 1,933,461. This support positions

the coils of wire in spaced relationship respecting the entire inside of the pot 1, whereby the gases enclosed by the latter may circulate more freely.

A first closure 8 is laid on the lower closure 5 seat 2 and a second closure 9 is laid on the upper seat 3. Both of these closures may be concentrically apertured so as to permit the insertion of a thermocouple 10 into the pot. It is to be noted that both the closures 8 and 9 are so constructed and arranged that both may be sealed with granular material.

In following the method described, the material positioned by the shell 4 may be any granular or porous material that is high in carbon. The 15 granular material which seals the closure 8 should also be of a carbonaceous character. The upper closure 9 may be sealed with a metallic oxide or any suitable refractory, whereby it functions to protect the carbonaceous material sealing the lower closure 8 from the furnace atmosphere.

I claim:

A method of pot annealing articles, including arranging articles to be annealed in substantially 25 annular formation in a container in spaced relation from the walls and ends of said container to provide gas passages interiorly and exteriorly of said articles, disposing carbonaceous material within said passage exteriorly of said articles. 30 sealing said container, applying heat to said container to anneal said articles, said passage exteriorly of said articles establishing a higher temperature zone and said passage interiorly of said articles establishing a lower temperature zone, 35 and circulating the atmosphere gases enclosed by said container upwardly through said higher temperature zone by the inherent expansion thereof, thereby carburizing said gases within said higher temperature zone, and circulating 40 said gases downwardly through said lower temperature zone by the relative contraction of said gases, thereby exposing said articles to the ascending carburized gases within said container.

CARL J. TOLL.